

Aug. 7, 1945.

W. H. HEATON

2,381,590

SHOE STIFFENER

Original Filed May 10, 1943



**Fig. 1**



**Fig. 2**

INVENTOR.

Walter H. Heaton.  
BY *Kenway & Witter.*  
*attys*



are set for 0.090 to 0.160 inch. The sheets leaving the calendering operation will be 0.045 to 0.080 inch in thickness. The surface next the calender roll on each sheet has imparted to it a relatively hard, smooth and compressed appearance whereas the inner surfaces of the sheets which contact each other remain relatively rough, porous and spongy with a mat finish.

In Fig. 1 the novel calendering step of my process is suggested. Two superposed sheets 12 and 13 are shown as passing through the calender rolls 10 and 11. The sheets 12 and 13 have been prepared as above described and are presented to the calender rolls substantially dry, but containing a small residue of solvent. The inner surfaces of the sheets 12 and 13 mat together as the sheets pass between the rolls while their outer surfaces are subjected to direct ironing engagement of the rolls. In Fig. 2 a fragment of the finished sheet material is indicated on a greatly magnified scale, the surface 15 being the porous spongy surface which has been cushioned in the calendering operation and the surface 14 being the relatively smooth compact surface formed by the direct engagement of the calender rolls.

Another advantage of my improved process is that it obviates all danger of spoiling the stock by over-doing the calendering operation. It has happened heretofore that by too close setting of the calender rolls or by calendering the stock while it contains too much residual solvent surfaces have been formed in the finished material which are so compact as to prevent the proper absorption of solvent in the conditioning step. By my improved process, however, one surface must of necessity be porous and absorbent regardless of such irregularities in the manufacturing pro-

cedure. Cellulose acetate and cellulose nitrate are the best stiffening compound in the form of a colloidal dispersion now known to me for purposes of my invention but I contemplate the employment of any other cellulose derivative having their characteristics.

The present application is a division of my prior application Serial No. 486,321, filed May 10, 1943, wherein I have claimed the method herein disclosed of making shoe stiffener material.

Having thus disclosed my invention and described in detail one manner of putting it into practice I claim as new and desire to secure by Letters Patent:

1. Shoe stiffener material comprising a double napped flannel saturated with a colloidally dispersed stiffening compound and having a relatively rough mat-finished surface on one side and having its nap laid down in a relatively smooth compact surface on the other side.

2. A box toe blank comprising a fabric base impregnated with a colloidally dispersed stiffening compound and having one mat-finished surface which is spongy and which will quickly absorb liquid solvent and bond firmly to cement, the other surface being ironed smooth and relatively slow in absorbent capacity.

3. A box toe blank comprising a woven fabric base impregnated with a colloidally dispersed 30 stiffening compound, selected from the group, cellulose acetate and cellulose nitrate and having one surface which is relatively non-absorbent, firm and compact and the other a mat finish surface spongy and highly absorbent of liquid solvent, the blank as a whole being limited in its absorbent capacity by its said compact surface portion.

WALTER H. HEATON.